

# United States Patent Office

3,006,741

Patented Oct. 31, 1961

1

3,006,741

## MOTOR FUELS

Frederick K. Kawahara, Park Forest, Ill., assignor to Standard Oil Company, Chicago, Ill., a corporation of Indiana  
No Drawing. Filed Mar. 31, 1958, Ser. No. 724,930  
12 Claims. (Cl. 44—66)

The present invention relates to stabilized light hydrocarbon distillates, and more particularly to a new and useful combination of additives for stabilizing motor fuels against oxidative gum formation. The invention provides a method of stabilizing hydrocarbon motor fuels which are derived at least in part from the thermal cracking of petroleum hydrocarbons.

Petroleum products, for example, motor fuels for spark-ignition internal combustion engines, naphthas, jet fuels, diesel fuels, fuel oils, etc. are normally susceptible to the formation of insoluble tars or gums upon exposure to the oxygen in air. This gum formation is particularly severe when petroleum products are derived, or contain constituents which are derived, from the thermal cracking of high boiling petroleum hydrocarbons. Olefinic materials, in particular diolefins and higher polyolefins, are associated with gum formation and are invariably found in commercial motor fuels which contain blends of thermally cracked gasoline. When motor fuels are to be maintained in storage for any considerable period, it is the practice to incorporate in such fuels an additive to inhibit gum formation.

An object of the present invention is to provide light hydrocarbon distillate fuels resistant to oxidative gum formation. Another object of the invention is to provide oxidation-stable hydrocarbon motor fuels which are derived at least in part from the thermal cracking of petroleum hydrocarbons. Still another object of the invention is to provide hydrocarbon motor fuels which are made resistant to oxidative gum formation by the incorporation of conventional oxidation inhibitors and a new synergist therefor. Other and more particular objects and advantages of the invention will become apparent from the following description.

In accordance with the objects above it has now been discovered that light hydrocarbon distillate fuels, particularly motor fuels and more particularly those distillates derived from thermal cracking of petroleum hydrocarbons, which are normally susceptible to oxidative gum formation, may be stabilized by incorporating therein a small but sufficient amount of a conventional para-phenylene diamine inhibitor and a perfluoroalkyl-amido-tertiary-amine synergist. Both the inhibitor and synergist are employed in amounts from about 0.001% to about 1.0%, and preferably from 0.001 percent to 0.01 percent by weight. The perfluoroalkyl-amido-tertiary-amines suitable for the present purpose have the general structural formula



in which the perfluoroalkyl group contains from 4 to 12 carbon atoms, the alkylene group contains from 1 to 6 carbon atoms, and the N-alkyl substituents contain from 1 to 6 carbon atoms, all ranges being inclusive.

Para-phenylene diamines are well known anti-oxidants and are widely used by the petroleum refining industry. These materials are typified by unsubstituted para-phenylene diamine, N-sec-butyl-paraphenylene diamine, N,N'-di-sec-butyl-para-phenylene diamine, N-t-butyl-para-phenylene diamine, N-hexyl-para-phenylene diamine and N-dodecyl-para-phenylene diamine. The N,N'-di-

2

butyl-para-phenylene diamine is an exceptionally effective inhibitor and is commercially available under the trademarks "du Pont No. 22" and "UOP No. 5."

The perfluoroalkyl-amido-tertiary-amines which have been found to possess an extraordinary synergism in the presence of para-phenylene diamines have been described in such publications as Blake et al., "Perfluoroalkyl Surface Active Agents for Hydrocarbon Systems," presented before the Division of Petroleum Chemistry, American Chemical Society, New York Meeting, September 11, 1954. The paper was published by the American Chemical Society in a booklet, "General Papers No. 32," September 11-17, 1954. The perfluoroalkyl-amido-tertiary-amines may be prepared by reacting the corresponding perfluoroalkyl carboxylic acid with the corresponding N,N-dialkyl-alkylene diamine; in turn the perfluoroalkyl carboxylic acids are obtained by the electrochemical fluorination of aliphatic carboxylic acids in anhydrous hydrofluoric acid according to the procedure of Kauck et al., Ind. Eng. Chem., vol. 43, No. 10, pp. 23-32, October 1951.

Perfluoroalkyl-amido-tertiary-amines alone have no detectable inhibiting effect on oxidative gum formation, but require that the phenylene diamine be conjointly present. To illustrate the surprising synergistic effect of perfluoroalkyl-amido-tertiary-amines on para-phenylene diamine inhibitors, two series of runs were conducted. In the first series, a thermally cracked heavy naphtha was employed as the oxidation-unstable hydrocarbon distillate base stock, and a para-phenylene diamine inhibitor and a perfluoroalkyl-amido-tertiary-amine synergist were incorporated therein, first independently and then in combination. As a measure of the tendency toward gum formation, the respective samples were exposed to the test conditions of ASTM 873-49 for four hours, and the gum contents at the end of this period were determined by the method of the test. Also in this first series several other perfluoroalkyl-amido compounds, the tetraalkyl ammonium halides, were tested and were found not to possess the synergistic properties of the tertiary amines claimed.

### Example I

An unstabilized thermal heavy naphtha was tested according to the above procedure. At the end of four hours it formed 83.5 milligrams of insoluble gum.

### Example II

A sample of the above naphtha was inhibited with 0.0027% by weight of du Pont No. 22, or N,N'-di-sec-butyl-para-phenylene diamine, without the perfluoroalkyl-amido-tertiary-amine. In four hours it formed 31.4 milligrams of gum, or a reduction of only 62.5 percent.

### Example III

The thermal naphtha and 0.0027% of perfluoroheptyl-CONH-propylene-N-dimethyl, without any para-phenylene diamine inhibitor, was tested. The gum formed was 92.9 milligrams, or an actual increase of 10% above Example I where the naphthas contained no additives.

### Example IV

In accordance with the invention, the thermal naphtha was inhibited with 0.0027% of du Pont No. 22 (N,N'-di-sec-butyl-para-phenylene diamine) and 0.0027% of perfluoroheptyl-CONH-propylene-dimethyl. At the end of the four hour test period the sample had deposited only 6.2 milligrams of gum. This is only 7.5% of the gum deposited by the untreated naphtha in Example I and is 80% less gum than formed by inhibition with a para-phenylene diamine inhibitor alone. In other words,

the phenylene diamine is rendered five times more effective, or, in the presence of the synergist, only one-fifth the amount of para-phenylene diamine inhibitor need be employed to attain the same degree of oxidation stability.

*Examples V and VI*

To compare perfluoroalkyl-amido-tertiary-amines with perfluoroalkyl-amido-tetraalkyl ammonium halides, the compound perfluoroheptyl-CONH-propylene-N(CH<sub>3</sub>)<sub>3</sub>I was tested both alone and in combination with a para-phenylene diamine. At the 0.0027% concentration level, the perfluoroalkyl-amido-tetraalkyl ammonium halide alone gave 120.8 milligrams of gum, or approximately 45% more than the thermal naphtha without any additives. The halide, rather than being a synergist for para-phenylene diamine proved antagonistic, and a naphtha containing 0.0027% each of the iodide and du Pont No. 22 deposited 151.2 milligrams of gum.

*Examples VII and VIII*

The compound perfluoroheptyl-CONH-propylene-N(CH<sub>3</sub>)<sub>3</sub>C<sub>10</sub>H<sub>21</sub>Br (referred to as the "bromide") when used alone with thermal naphtha greatly promoted gum formation, there being deposited 449.0 milligrams at the end of four hours at the 0.0027% concentration level. As a synergist for N,N'-di-sec-butyl-para-phenylene diamine (du Pont No. 22, both at 0.0027% concentration) it was somewhat better than the iodide of Examples V and VI. In four hours, 66.8 milligrams of gum were deposited, or about 11 times the amount of gum that was formed in using the combination of the instant invention (Example IV).

In a second series of eight additional tests the surprising promotional effect of perfluoroalkyl-amido-tertiary-amines on para-phenylene diamines were further studied. The base stock in each case was a synthetic mixture consisting of 2.5 parts by volume of 2,3-dimethyl butadiene-1,3 in 100 parts of normal heptane. Dimethyl butadiene was selected as it typically represents unstable diolefinic hydrocarbons present in thermally cracked petroleum fractions, and its susceptibility to oxidative gum formation renders it an excellent test stock for quantitative as well as qualitative comparisons of additives. In each run the amount of the additive employed was 0.0027% by weight.

*Examples IX and X*

The synthetic stock described above, in the absence of any additive, was studied under the conditions of the ASTM 873-49 gum determination test. At the end of four hours, 631.0 and 635.7 milligrams of gum were formed.

*Examples XI and XII*

In two tests, the stock containing 0.0027% of the perfluoroalkyl-amido-tertiary-amine, perfluoroheptyl-CONH-propylene-N-dimethyl, in the absence of a phenylene diamine inhibitor, formed 603.8 and 468.0 milligrams of gum in four hours. This indicates a very slight improvement, if any, in oxidative gum stability caused by the synergist alone.

*Examples XIII and XIV*

A sample of the dimethyl butadiene-normal heptane mixture was inhibited with the commercial phenylene diamine, N,N'-di-sec-butyl-para-phenylene diamine (du Pont No. 22), in the amount of 0.0027%. In two tests of four hours each, 23.6 milligrams of gum was formed in each case.

*Examples XV and XVI*

A mixture of the dimethyl butadiene normal heptane hydrocarbon with commercial N,N'-di-sec-butyl-para-phenylene diamine together with the synergist perfluoro-

heptyl-CONH-propylene-N-dimethyl was tested by the standard ASTM method. In four hours only 7.5 milligrams and 13.5 milligrams of gum were formed, for an average of 10.5 milligrams—or a 56.7% reduction of

5 the amount formed with anti-oxidant alone.

In similar manner other perfluoroalkyl-amido-tertiary-amines may be used, and these include for example perfluoro-N-butyl-CONH-ethylene-N-methyl-ethyl, perfluoroisooctyl-CONH-isobutylene-N-diethyl, perfluorononyl-CONH-hexylene-N-dibutyl, and perfluorododecyl-CONH-propylene-N-dimethyl.

The data in the above sixteen runs demonstrate that the combination of para-phenylene diamine anti-oxidant with perfluoroalkyl-amido-tertiary-amines is vastly superior to the anti-oxidant itself in inhibiting oxidative degradation or gum formation of petroleum distillates. The thermally cracked naphtha and the synthetic dimethyl butadiene heptane mixtures tested are representative of the most unstable petroleum hydrocarbons and the data 15 clearly illustrate the advantages obtainable with the combination according to the invention.

Because the perfluoroalkyl-amido-tertiary-amines are sparingly soluble in hydrocarbons, special methods are employed to incorporate the synergists into the distillate 20 stock. The synergist may be mixed with a lower alkanol such as normal propyl alcohol or normal butanol and the resulting solution added to the hydrocarbon; n-butanol method was employed in the examples above. Alternatively, the perfluoroalkyl-amido-tertiary-amine may be 25 dissolved or dispersed in water, the aqueous solution admixed with the hydrocarbon, and the mixture heated to drive off the water. This latter method is very advantageously employed prior to a distillation step in the production of the petroleum stock. Since light petroleum 30 distillates are conveniently produced by thermal or catalytic cracking or by special conversion processes such as reforming, catalytic alkylation, or polymerization, all of which include a final stabilization step, and aqueous mixture of perfluoroalkyl-amido-tertiary-amine synergist, 35 with or without the inhibitor, is advantageously incorporated into the stock before stabilization, and the water removed along with the light ends. The light distillates have an initial boiling point of about 90° F. to about 200° F., those in the gasoline or motor fuel range boil 40 from about 100 to 400° F., and those in the diesel fuel and heating oil range boil from about 350° F. to about 45 700° F., more or less.

Aside from their herein demonstrated synergistic effects in promoting phenylene diamine inhibitors, perfluoroalkyl-amido-tertiary-amines are known to have another advantageous property with respect to petroleum distillates. It is reported in the Blake et al. publication previously noted that perfluoroalkyl-amido-tertiary-amines in a concentration of about 0.001 percent or more based on hydrocarbon 50 reduce the surface tension of the mixture by about 50%, thus making for improved efficiency in distillation of hydrocarbons containing these materials. Moreover, and of special commercial significance, perfluoroalkyl-amido-tertiary amines are highly surface active; a few thousands of a percent of these compounds in hydrocarbon 55 is capable of reducing the rate of hydrocarbon evaporation by 75 to 85%. This is especially advantageous when one considers that the usual evaporation loss of volatile petroleum distillates such as motor fuels both during storage and in filling the consumers gasoline 60 tank may amount to several volume percent. Thus, in addition to improving oxidation resistance, or in providing identical oxidation resistance at greatly reduced phenylene diamine concentrations, the perfluoroalkyl-amido-tertiary- 65 amines give the added benefits of facilitating distillation and of reducing evaporation loss. Where evaporation loss is considered a major problem, the perfluoroalkyl portion of the synergist is preferably highly branched, rather than straight chain, so as to provide a large molecular volume, 70 and such branching may conveniently be attained by em-

ploying perfluoroalkyl carboxylic acids derived from alcohols produced by the well known Oxo reaction.

The perfluoroalkyl-amido-tertiary-amine and para-phenylene diamine mixture of the present invention can be used in combination with conventional petroleum additives such as tetraethyllead, alkyl halide scavengers, anti-wear agents, agents for inhibiting spark plug fouling, corrosion inhibitors, de-icers, etc.

Percentages given herein and used in the appended claims are by weight unless otherwise stated.

While the invention has been described and illustrated by way of preferred embodiments thereof, it will be apparent to those skilled in the art that variations and modifications may be made without departing from the scope of the present invention as defined by the appended claims.

I claim:

1. A stabilized hydrocarbon light distillate normally susceptible to oxidative gum formation, containing in combination from about 0.001% to 1.0% of a para-phenylene diamine inhibitor selected from the group consisting of para-phenylene diamine, N-secbutyl-para-phenylene diamine, N,N'-di-secbutyl-para-phenylene diamine, N-t-butyl-para-phenylene diamine, N-hexyl-para-phenylene diamine and N-dodecyl-para-phenylene diamine and from about 0.001 to 1.0% of a perfluoroalkyl-amido-tertiary-amine synergist having the general structure



in which the perfluoroalkyl group contains from 4 to 12 carbon atoms, the alkylene group contains from 1 to 6 carbon atoms and the N-alkyl substituents contain from 1 to 6 carbon atoms.

2. The stabilized hydrocarbon light distillate of claim 1 in which the perfluoroalkyl-amido-tertiary-amine is perfluoroheptyl-CONH-propylene-N-dimethyl.

3. A stabilized petroleum hydrocarbon motor fuel obtained at least in part by thermal cracking of petroleum hydrocarbons, and normally susceptible to oxidative gum formation, containing in combination from about 0.001% to 1.0% of a para-phenylene diamine inhibitor selected from the group consisting of para-phenylene diamine, N-secbutyl-para-phenylene diamine, N,N'-di-secbutyl-para-phenylene diamine, N-t-butyl-para-phenylene diamine, N-hexyl-para-phenylene diamine and N-dodecyl-para-phenylene diamine and from about 0.001% to 1.0% of a perfluoroalkyl-amido-tertiary-amine synergist having the general structure



in which the perfluoroalkyl group contains from 4 to 12 carbon atoms, the alkylene group contains from 1 to 6 carbon atoms and the N-alkyl substituents contain from 1 to 6 carbon atoms.

4. The stabilized hydrocarbon motor fuel of claim 3 in which the perfluoroalkyl-amido-tertiary-amine is perfluoroheptyl-CONH-propylene-N-dimethyl.

5. A stabilized hydrocarbon motor fuel of the gasoline boiling range, adapted for spark-ignition internal combustion engines and derived at least in part by thermal cracking of petroleum hydrocarbons, containing from about 0.001% to about 1.0% of a para-phenylene diamine oxidation inhibitor selected from the group consisting of para-phenylene diamine, N-secbutyl-para-phenylene diamine, N,N'-di-secbutyl-para-phenylene diamine, N-t-butyl-para-phenylene diamine, N-hexyl-para-phenylene diamine and N-dodecyl-para-phenylene diamine and from about 0.001% to about 1.0% of a perfluoroalkyl-

amido-tertiary-amine synergist having the general structure



in which the perfluoroalkyl group contains from 4 to 12 carbon atoms, the alkylene group contains from 1 to 6 carbon atoms, and the N-alkyl substituents contain from 1 to 6 carbon atoms.

6. The hydrocarbon motor fuel of claim 5 in which the perfluoroalkyl-amido-tertiary-amine is perfluoroheptyl-CONH-propylene-N-dimethyl.

7. The method of stabilizing a hydrocarbon light distillate normally susceptible to oxidative gum formation which comprises incorporating therein from about 0.001 to 1.0% of a para-phenylene diamine inhibitor selected from the group consisting of para-phenylene diamine, N-secbutyl-para-phenylene diamine, N,N'-di-secbutyl-para-phenylene diamine, N-t-butyl-para-phenylene diamine, N-hexyl-para-phenylene diamine and N-dodecyl-para-phenylene diamine and from about 0.001% to 1.0% of a perfluoroalkyl-amido-tertiary-amine synergist having the general structure



in which the perfluoroalkyl group contains from 4 to 12 carbon atoms, the alkylene group contains from 1 to 6 carbon atoms, and the N-alkyl substituents contain from 1 to 6 carbon atoms.

8. The method of claim 7 in which the perfluoroalkyl-amido-tertiary-amine is perfluoroheptyl-CONH-propylene-N-dimethyl.

9. A stabilized hydrocarbon light distillate normally susceptible to oxidative gum formation, containing in combination from about 0.001% to 1.0% N,N'-di-secbutyl-para-phenylene diamine and from 0.001% to 1.0% of a perfluoroalkyl-amido-tertiary amine having the general formula



in which the perfluoroalkyl group contains from 4 to 12 carbon atoms, the alkylene group contains from 1 to 6 carbon atoms and the N-alkyl substituents contain from 1 to 6 carbon atoms.

10. The stabilized hydrocarbon light distillate of claim 9 in which the perfluoroalkyl-amido-tertiary amine is perfluoroheptyl-CONH-propylene-N-dimethyl.

11. A stabilized petroleum hydrocarbon motor fuel obtained at least in part by thermal cracking of petroleum hydrocarbons, and normally susceptible to oxidative gum formation, containing in combination from about 0.001% to 1.0% of an N,N'-di-secbutyl-para-phenylene diamine and from about 0.001% to 1.0% of a perfluoroalkyl-amido-tertiary-amine synergist having the general structure



in which the perfluoroalkyl group contains from 4 to 12 carbon atoms, the alkylene group contains from 1 to 6 carbon atoms and the N-alkyl substituents contain from 1 to 6 carbon atoms.

12. A stabilized hydrocarbon motor fuel of the gasoline boiling range, adapted for spark-ignition internal combustion engines and derived at least in part by thermal cracking of petroleum hydrocarbons, containing from about 0.001% to about 1.0% of N,N'-di-secbutyl-para-phenylene diamine and from about 0.001% to

about 1.0% of a perfluoroalkyl-amido-tertiary-amine synergist having the general structure

in which the perfluoroalkyl group contains from 4 to 12 carbon atoms, the alkylene group contains from 1 to 6 carbon atoms, and the N-alkyl substituents contain from 1 to 6 carbon atoms.

10

References Cited in the file of this patent

UNITED STATES PATENTS

|           |                 |                |
|-----------|-----------------|----------------|
| 2,680,717 | Little          | June 8, 1954   |
| 2,700,612 | Chenicek        | Jan. 25, 1955  |
| 2,734,808 | Biswell         | Feb. 14, 1956  |
| 2,764,603 | Ahlbrecht       | Sept. 25, 1956 |
| 2,824,884 | Barnhart et al. | Feb. 25, 1958  |